

## UNITED STATES PATENT OFFICE

1,949,529

## REFINING OF STEEL

Vere B. Browne, Brackenridge, Pa., assignor to  
Allegheny Steel Company, Brackenridge, Pa., a  
corporation of Pennsylvania

No Drawing. Application April 26, 1930,  
Serial No. 447,770

9 Claims. (Cl. 75—27)

This invention relates to the refining of steel and especially to a new and novel method of effecting such refining by invoking and utilizing the principles of physical chemistry.

5 It has been generally considered that the reactions taking place in a furnace are purely chemical and that in order to remove impurities from the steel it has been assumed that a chemical union must take place so that the impurities are 10 either oxidized or reduced and thus put in a condition in which they can be isolated or collected and removed.

While this is true as far as it goes, I have discovered that certain impurities can be removed 15 without depending solely on a chemical union, but rather by changing the solution pressures of the two liquids (steel and slag) so that the utilized tendency or effect is a physical rather than a chemical one.

20 One of the objects of my invention, therefore, is the refining of steel by a change of solution pressure, thus utilizing the principles of physical chemistry.

Another object of my invention is to refine steel 25 of any type having a supernatant slag by causing the oxids dissolved in the steel to migrate to the slag.

A further object of my invention is the conversion of oxids to silicates in the slag by adding in 30 effect the  $\text{SiO}_2$  radical to the slag in excess.

Other and further objects will be understood by those skilled in this particular art.

I have discovered that steel can be produced 35 free from oxids, such as  $\text{FeO}$  and  $\text{MnO}$  and the like, even under a slag extremely high in oxids provided that the solution pressure can be changed so that the oxids migrate or tend to migrate from the metal to the slag and provided that there is an acid radical present to combine 40 with the oxids. This is, I believe, a logical explanation of the difference between acid and basic steel.

For example, in the making of silicon steel in 45 an electric or open hearth furnace, it is desired to have the carbon content as low as possible, but when the carbon content has been reduced to say about .02% the slag will contain, many times, as much as about 35%  $\text{FeO}$  and the metal will be practically saturated with oxids. 50 When silicon is added to such steel the silicon reduces the  $\text{FeO}$  and is itself oxidized to silica ( $\text{SiO}_2$ ) which is entrapped in the metal in the form of an emulsion. Even the removal of the slag does not help materially under such conditions as the metal still contains dissolved oxids.

I have discovered further that these oxids can be removed by changing the composition of the slag and so changing the solution pressures of the two liquids, thus causing the oxids to migrate to the slag instead of remaining in the metal. 60 This phenomenon may be termed "mass action equilibrium".

For example, a slag consisting of



will have a pressure relation to the metal which will cause the free  $\text{FeO}$  to migrate to the metal in which it becomes dissolved, whereas a slag consisting of



will have a relation to the metal which will cause the  $\text{FeO}$  to migrate to the slag, where it chemically unites with the  $\text{SiO}_2$ .

I have discovered, therefore, that it is possible to remove oxids completely from low carbon steels such as are used, for example, in the manufacture of transformer sheets by adding sand to the slag at the end of the operation in an amount sufficient to more than combine with all the  $\text{MnO}$  and  $\text{FeO}$  present. This will effect a change in 80 the solution pressure and the dissolved oxids will be liberated from the metal to combine with the excess silica. It is known that metallic silicates dissolve in each other when melted and also that they dissolve oxids of metals, but they do not 85 dissolve metals or reduced substances.

In case one prefers to remove the slag entirely the same result can be obtained by replacing the original slag with a slag composed of  $\text{CaO}$  and  $\text{SiO}_2$  but with a liberal excess of  $\text{SiO}_2$  over 95 and above that amount calculated to combine with the amount of dissolved oxids estimated to be present.

Experimentation has proved not only the accuracy of the above considerations, but that valuable results are secured economically and efficiently.

In general, when acid radical is present in sufficient quantities, all the basic substances in the slag are satisfied and hence the slag has a further capacity for attracting to itself additional oxids, which are likewise satisfied, and the migration continues. If the slag has an excess of acid radical it is understood that all the oxids will be removed from the steel.

The process is applicable to any kind of steel and may be used, for example, in connection with silicon steel or chrome alloys, but it is not limited thereto.

5 What I claim as new and desire to secure by Letters Patent is:—

1. In the process of refining steel containing dissolved basic oxids and having a surface slag thereon, adding in effect the  $\text{SiO}_2$  radical in excess of that theoretically necessary to convert all said dissolved oxids into silicates, bringing about a change in the relative solution pressures of steel and slag so as to set up a migratory tendency of the dissolved oxids from the steel to the slag, said oxids being converted in said slag into corresponding silicates, said excess  $\text{SiO}_2$  radical in said slag maintaining said slag free from uncombined oxids other than  $\text{SiO}_2$  and hence preventing a premature equilibrium or a reversal of the migration.
- 10 2. In the process of refining steel containing dissolved basic oxids and having a slag thereon, causing the dissolved oxids to migrate from said steel to said slag by adding in effect to said slag an amount of acid radical over and above the combining equivalent of the oxids, said oxids there combining with the chemical equivalent of acid radical and maintaining said slag free from uncombined oxids other than those of the acid radical itself.
- 15 3. In the process of refining steel containing dissolved basic oxids and having a slag thereon, causing all the dissolved oxids to migrate from said steel to said slag by adding to said slag in effect the  $\text{SiO}_2$  radical in excess of the combining equivalent of said oxids, said oxids there combining with an equivalent amount of said  $\text{SiO}_2$  radical.
- 20 4. In the process of refining steel containing dissolved basic oxids and having a slag thereon, causing all the dissolved oxids to migrate from said steel to said slag by adding to said slag in effect the  $\text{SiO}_2$  radical in excess of the combining equivalent of said oxids, said oxids there combining with an equivalent amount of said  $\text{SiO}_2$  radical producing corresponding silicates and maintaining said slag free from uncombined oxids other than those of the acid radical itself.

50

55

60

65

70

75

5. A process of removing dissolved basic oxids from low carbon steels containing the same and having a supernatant slag, comprising adding sand to the slag at the end of the steel-making operations in an amount more than sufficient to combine with said dissolved oxids.

6. A process of removing basic oxids entrapped in molten steel containing the same and having a supernatant slag, comprising liberating said oxids from said steel and causing them to migrate to said slag where they are chemically combined by adding in effect to said slag the  $\text{SiO}_2$  radical in excess of the combining equivalent of said oxids.

7. In the manufacture of steel containing dissolved iron and manganese oxids and having a supernatant slag, the steps of adding acid radical  $\text{SiO}_2$  in effect in excess of the combining equivalent of said oxids to said slag, causing said iron and manganese oxids to migrate to said slag and to combine with a portion of said acid radical  $\text{SiO}_2$  to form iron and manganese silicates which remain in and become a part of said slag.

8. A physico-chemical method of treating steel containing dissolved or entrapped oxids and having a supernatant slag involving causing said oxids to physically pass from said steel to said slag by an adjustment of solution pressures of steel and slag to bring about such transference by adding  $\text{SiO}_2$  in excess of the combining equivalents of the oxids and causing said so-transferred oxids to chemically unite with a portion of said slag specially added for such purposes.

9. A physico-chemical process of refining molten steel which has a supernatant molten slag thereon, both steel and slag containing dissolved and entrapped oxids, comprising adding available  $\text{SiO}_2$  to the slag in an amount more than sufficient to combine with all such oxids, thus converting oxids in the slag to corresponding silicates, setting up a physical migration of oxids from steel to slag, converting to corresponding silicates such migrated oxids, and preventing premature equilibrium or reversal of the aforesaid action.

VERE B. BROWNE.

120

110

115

100

95

85

80

90

140

135

140

145

150